

April 25, 1944.

J. L. PETRIE

2,347,280

DIAMOND DRESSING TOOL AND METHOD OF  
DETERMINING DIAMOND SIZES THEREFOR  
Filed July 12, 1941



## UNITED STATES PATENT OFFICE

2,347,280

## DIAMOND DRESSING TOOL AND METHOD OF DETERMINING DIAMOND SIZES THEREFOR

John L. Petrie, Detroit, Mich., assignor to Wheel Trueing Tool Company of Delaware, Detroit, Mich., a corporation of Delaware

Application July 12, 1941, Serial No. 402,054

1 Claim. (Cl. 125--39)

This invention relates to diamond tools for dressing abrasive wheels wherein the size of the diamonds in the tools is selected in accordance with the characteristics of the abrasive wheel to be dressed.

More specifically this invention relates to diamond wheel dressing tools having the diamonds thereof especially selected for carrying out most effectively the dressing of specific types or groups of abrasive wheels for which the tools are intended.

In my copending application Serial No. 349,513, entitled: "Diamond dressing tool and method of dressing grinding wheels," filed August 2, 1940, now U. S. Patent No. 2,254,392, issued September 2, 1941, there is described and claimed diamond dressing tools having small diamonds ranging from one-quarter carat down to 0.01 carat, or down to a small size so as to be just large enough not to pass through a 200-mesh screen. These dressing tools have the diamonds thereof arranged in a single plane. The single plane of diamonds is preferably composed of a plurality of tiers having the diamonds thereof in overlapping relation. For example, one tier of diamonds can contain three or four diamonds, while the next tier can contain two or three diamonds. In this manner the diamonds are staggered and, as the same become worn, a new diamond will come into operation before the worn diamonds are completely spent.

I have found that these small diamond tools are especially adapted for use in trueing that class of precision grinding abrasive wheels whose grain sizes are 30 mesh or finer but not appreciably finer than 120 mesh. That is, the grains of such wheels are sized so that they will pass through screens not coarser than 30 mesh per linear inch, nor finer than 120 mesh per linear inch. Coarse grain wheels below size 30 grain do not need to be trueed with accuracy, since they are generally used for snagging or roughing operations where precision grinding finish is not required. On the other hand, fine grain wheels of above 120 size grain require dressing tools with diamonds large enough to resist abrasion but, if the diamonds are too large in relation to the fine grain, they will tend to crush the grains and "close up" or "glaze" the wheel. To have good grinding characteristics the wheel must be "open" or "sharp."

According to the present invention, diamond sizes for such small diamond tools are positively controlled in accordance with the characteristics of the abrasive wheel or group of abrasive wheels

to be acted on by the tools and particularly the group of abrasive wheels lying within that class having grain sizes not appreciably coarser than size 30 nor finer than size 120. The efficiency of the diamond tools is greatly enhanced since each tool is specifically designed or engineered for a particular job and, if the characteristics of the abrasive wheel are known, this invention now furnishes the correct dressing tool for the wheel.

Therefore, the diamond tools of this invention not only utilize small diamonds in place of the heretofore-required large diamonds but, in addition, the small diamonds in the tools are so selected as to most effectively perform on particular types of abrasive wheels.

The characteristics of the abrasive wheels controlling the sizes of the diamonds includes the following:

- (1) Grain size of abrasive grit.
- 20 (2) Hardness of wheel (holding power of bond).
- (3) Nature and hardness of grit.

I have discovered that the diamond size in wheel dressing tools should increase in direct proportion to the grain size of the abrasive wheel grit. I have found that the size or diameter of the wheel itself is not controlling.

I have further found that the "hardness" of the abrasive wheel is also an important factor in determining optimum diamond sizes since the bond grade or grit holding power, to a great extent, determines the wear on the diamond itself. The hardness of the wheel is determined by the grade of the bonding material and the amount of bond as compared with the amount of grains. In any given type of bonding material such as a vitrified bond, for example, the wheel is "harder" as the amount of bond relative to the amount of grain increases. Thus the more bond, the greater the holding power for the grits. In the harder grinding wheels, while the abrasive grits are not necessarily harder, there is more bonding agent holding the grits together and it is therefore necessary in the successively greater bonded abrasive wheels to use successively larger diamonds, much as it is necessary to increase the size of the diamond in accordance with the coarseness of the grain or grit in each wheel.

The nature and hardness of the grits or grains themselves should also be taken into consideration. For example, the dressing of a silicon carbide grit wheel requires a dressing tool with larger diamonds than those necessary in a tool for dressing an aluminum oxide grit wheel even

though the two wheels have the same grit size and wheel "hardness." This is probably not only necessitated by the greater hardness of the silicon carbide grits but may be partly due to the greater heat retention properties of the silicon carbide. Silicon carbide grits retain more heat and are thus heated more than aluminum oxide grits when being cut by the dressing tool and therefore cause increased heating of the diamonds. The aluminum oxide grits throw off the heat generated on cutting. Therefore the diamonds must be larger as the heat retention properties and hardness of the grits increases so as to be able to resist the increased heat.

It is, then, an object of this invention to selectively size diamonds in wheel dressing tools in accordance with characteristics of abrasive wheels to be dressed thereby.

A further object of the invention is to provide diamond dressing tools with small sized diamonds selected to perform best on certain types of abrasive wheels.

A further object of this invention is to provide diamond dressing tools which are engineered for the particular jobs which they are to perform.

A specific object of this invention is to provide diamond dressing tools having a plurality of small diamonds arranged in tiers in a single plane, so that they will line up one behind the other in substantially the same cutting track when acting on an abrasive wheel and wherein the size of the small diamonds is carefully selected in accordance with the characteristics of the abrasive wheels to be dressed thereby.

Another specific object of the invention is to selectively control the sizes of diamonds in diamond dressing tools in accordance with the grain size, grain hardness and bond characteristics of the abrasive wheel to be dressed by the tools.

A further specific object of this invention is to provide wheel dressing diamond tools with diamonds less than one-quarter carat and selectively sized in direct relation to the grain size of the abrasive wheels to be dressed thereby.

Other and further objects of this invention will become apparent to those skilled in the art from the following detailed descriptions of the annexed sheet of drawings which, by way of preferred example, illustrate the invention.

On the drawing:

Figure 1 is a fragmentary end elevational view, with parts broken away and in section, of a wheel dressing assembly illustrating the proper mounting in a holder of a dressing tool according to this invention.

Figure 2 is an enlarged fragmentary elevational view of a diamond dressing tool embodying my invention with parts broken away and in section to show the positioning of the diamonds.

Figure 3 is a top plan elevational view of the diamond dressing tool.

Figure 4 is a fragmentary sectional view taken substantially along the line IV-IV of Figure 3.

Figure 5 is a chart showing the relationship between the diamond sizes and grain sizes of abrasive wheels to be dressed by the tools of this invention.

As shown on the drawing:

In Figure 1 the reference numeral 10 designates generally a mounting for a grinding wheel 11. A tool holder 12 serves to hold a dressing tool 13 of this invention in dressing relationship to the surface of the grinding wheel. A set screw 14 fixedly secures the tool 13 in the holder.

The tool 13 is preferably provided with an off-

10 set end 15 so as to adapt it for use in a conventional type of tool holder.

As shown in Figures 2 to 4 the diamond dressing tool 13 comprises a cylindrical shank 16 from which extends the offset end 15 joined thereto by tapering shoulders 17. The end 15 has a rectangular shaped flat end face 18 when new but the particular form and shape of the tool is not critical.

The metal of the tool end 15 comprises a matrix in which are embedded a plurality of diamonds 19 which, according to the invention, are arranged in one or more tiers with the diamonds in each tier in substantial alignment. Three such tiers A, B and C are illustrated with the diamonds of the tiers in overlapping relation so that, as the diamonds in one tier become worn, the diamonds in the next successive tier come into cutting or dressing position. The diamonds preferably have their long axes parallel to the axis X-X of the tool end 15, as shown in Figure 2.

While it is not essential that the number of diamonds in the successive tiers be as shown, viz., 3, 2 and 3, this arrangement gives very desirable results, but the advantages of this arrangement can be realized also by employing a 4-3-4 combination as well as other combinations, such as 2-2-2; 3-3-3; and 4-4-4.

All of the diamonds lie in substantially a single plane and the tool is set in the holder 12 so that the plane of the diamonds is transverse to the axis of the wheel 11. In this position the diamonds in each tier follow in substantially the same cutting track and bring about a cutting rather than a crushing action on the grains of the abrasive wheel. As a result the surface of the abrasive wheel is freer and more open with less fine grit packed in between the grains.

The middle diamond indicated by the reference numeral 19M in Figures 2 and 3 is, as shown in Figure 1, positioned so that it lies on a radius line RL passing through the axis of the grinding wheel mounting 10.

According to previous standards it had been thought necessary in the dressing of grinding wheels that the size of the diamond should bear some fixed relation to the diameter and width of face of the wheels to be trued. For example with a wheel of six inches and under in diameter a half-carat diamond was generally considered necessary while with wheels as large as thirty-six and forty-two inches in diameter, it was considered necessary to use a diamond of six or eight carats respectively. Likewise, larger diamonds were considered necessary for dressing wheels with wide grinding faces than for wheels with narrower grinding faces.

I have now found that the diamond dressing tools of this invention can utilize small diamonds varying from a size just large enough to be retained on a 200-mesh screen up to one-quarter carat. The diamonds should preferably weigh between 0.01 and .25 carat, but the optimum weight of the diamond is controlled by the type of abrasive wheel on which the tool is to be used.

I have found that there is a definite relationship between optimum diamond size and the abrasive grain size of the abrasive wheel. Abrasive grains or grits are designated by numbers corresponding to the number of meshes per lineal inch of the screens through which they are graded. Thus a 36-grain wheel constitutes an abrasive wheel having abrasive grains or grits embedded therein which pass through a screen having 36 meshes per linear inch. The grains

are graded, however, so that they will not pass through the next size smaller screen.

I have also found that the "hardness" of the abrasive wheels as determined by the bond grade must be considered when determining the optimum diamond size for the dressing tool. For example vitrified bonded wheels are usually classified as soft, medium and hard, depending upon the amount of bond in the wheel as compared with the amount of grain or grit in the wheel. The same size abrasive grain in a hard vitrified wheel will require larger diamonds in the dressing tool than when the medium or soft vitrified wheel is used. The vitrified bond usually consists of a clay mixture subjected to sufficiently high temperature to fuse to a molten glass condition.

The hardness of the particular abrasive grain or grit likewise has some effect upon proper selection of diamond sizes. For example, aluminum oxide grains or grits are quite tough but are not as hard as silicon carbide grits. The silicon carbide grits, being harder and retaining more heat than the aluminum oxide grits, require larger sized diamonds than the aluminum oxide grits.

The aluminum oxide hard abrasive wheels best acted on by the dressing tools of this invention have grain sizes varying from 30 to 60 and, as shown in curve C, the diamond size should be within the range of .155 to .10 carat and decrease in direct proportion to the decrease in grain size.

The curves D, E and F relate to silicon carbide abrasive grains in soft, medium, and hard vitrified bonded wheels respectively. The silicon carbide soft wheels best trued by the tools of this invention have grain sizes varying from 60 to 120 and should be dressed with tools having the diamond sizes varying from .04 to .03 carat. The silicon carbide medium hard abrasive wheels best trued by the tools of this invention have grain sizes varying from 36 to 70 and should have the diamond size of the dressing tool vary from .085 to .05. The hard silicon carbide wheels best trued by the tools of this invention having grain sizes varying from 36 to 60 should have the diamond size of the dressing tool vary from .1975 to .16.

The curves A, B, C, D, E and F were plotted from actual data obtained as a result of comprehensive tests summarized in the following chart:

|                                         | Abrasive grain size |       |      |      |       |      |     |       |     |     |  |
|-----------------------------------------|---------------------|-------|------|------|-------|------|-----|-------|-----|-----|--|
|                                         | 30                  | 36    | 40   | 46   | 50    | 54   | 60  | 70    | 80  | 120 |  |
| Diamond carat sizes:                    |                     |       |      |      |       |      |     |       |     |     |  |
| Aluminum oxide soft wheels (curve A)    |                     | .05   | .045 | .04  | .0375 | .035 | .03 | .0225 |     |     |  |
| Aluminum oxide medium wheels (curve B)  |                     | .075  | .07  | .065 | .06   | .055 | .05 | .04   | .03 |     |  |
| Aluminum oxide hard wheels (curve C)    | .155                | .145  | .135 | .125 | .1175 | .11  | .10 |       |     |     |  |
| Silicon carbide soft wheels (curve D)   |                     |       |      |      |       |      | .04 | .0325 | .03 | .03 |  |
| Silicon carbide medium wheels (curve E) |                     | .085  | .08  | .075 | .07   | .065 | .06 | .05   |     |     |  |
| Silicon carbide hard wheels (curve F)   |                     | .1975 | .19  | .18  | .175  | .16  |     |       |     |     |  |

It should be noted, however, that the hardness of the abrasive grain does not determine the hardness of the grinding wheel itself. The grinding wheel may be made of very hard abrasive grits and still be considered a soft wheel if relatively small amounts of bond, compared with the amounts of grit, is used. A grinding wheel is considered hard when the retentive powers of the bonding material are great. If the grains of abrasive are easily broken out of the bond, the wheel is soft.

Since each abrasive wheel is marked by the manufacturer as to abrasive grain or grit size, bond grade (amount of bond), type of grit, wheel structure (relative grain spacing), and the like, all data necessary for selecting the proper dressing tool in accordance with this invention is available.

In Figure 5 the graph illustrates the relationship which I have discovered between correct diamond sizes for dressing tools and abrasive grain size, abrasive grain hardness and hardness of wheels to be dressed by the tools.

The curves marked A, B and C in the graph are plotted for aluminum oxide abrasive grit wheels in soft, medium, and hard vitrified bonded wheels respectively. The aluminum oxide soft wheels best acted on by the dressing tools of this invention have grain sizes varying from 36 to 70. As shown by curve A, the proper diamond sizes for the dressing operation should be within the range of .05 to .0225 carat and should decrease proportionally to the decrease in grain size.

The aluminum oxide medium hard wheels best acted on by the dressing tools of this invention have grain sizes varying from 36 to 80 and, as shown by curve B, the diamond sizes should be within the range of .075 to .03 carat, and decrease directly with the decrease in grain size.

From the above descriptions it will be apparent that this invention now provides diamond tools with a plurality of diamonds set in a single plane so as to line up one behind the other in substantially the same cutting track. The diamonds vary in size from .01 to .25 carat but are of uniform size in each tool. The sizes of the diamonds are selectively controlled in accordance with the nature of the abrasive wheel to be dressed by the tool. The size of the abrasive wheel grains or grits, the hardness of the wheel as determined by the amount of bond in the wheel, and the hardness of the grits themselves control the size of the diamond. The diamond sizes increase in substantially direct proportion to the increase in the grain size; increase in grain hardness; and increase in wheel hardness.

I claim as my invention:

The method of dressing abrasive grit grinding wheels of the class having abrasive grits of a size not appreciably coarser than size 30 nor finer than size 120 with a plurality of small diamonds which comprises determining the grit size of each wheel to be dressed, selecting substantially uniformly sized diamonds within a size range of .0225 to 0.1975 carat in accordance with the grit size of the wheel to be dressed to provide the smaller diamonds for the finer grit size wheels and the larger diamonds for the coarser grit size wheels and with the diamond sizes increasing in substantially direct proportion to the increase in grit size, holding a plurality of the thus selected substantially uniformly sized diamonds against the wheel of determined grit size for which the diamonds were selected in a plane substantially transverse to the axis of rotation of the wheel to simultaneously act on the wheel in substantially the same cutting track, and rotating the wheel.

JOHN L. PETRIE.